

March 3, 1942.

F. C. JACOBS

2,274,699

METALLIC FILAMENTOUS MATERIAL

Filed Feb. 2, 1940



INVENTOR

Frank C. Jacobs  
by Chinty and Wharton  
his attorneys

## UNITED STATES PATENT OFFICE

2,274,699

## METALLIC FILAMENTOUS MATERIAL

Frank C. Jacobs, New Kensington, Pa.

Application February 2, 1940, Serial No. 316,972

4 Claims. (Cl. 140—71)

My invention relates to devices and articles constructed of or including elastic filaments of metal, and more particularly to the elastic filaments used in the construction of such devices and articles. The invention consists in an improved filament structure.

The elastic filament of the invention is particularly designed for use in packings of the construction illustrated and described in my copending application for Letters Patent, Serial No. 316,973, filed February 2, 1940, but it also is adapted for a great number of other uses. For example, the filament provides (when properly woven, knitted, or otherwise fashioned into a fabric, or a cluster or bunch) a particularly effective scouring, buffing, or abrading instrumentality, which may be used in such devices as condenser tube cleaners, metal "sponges" for the cleansing of cooking utensils, and the like.

In the accompanying drawing I show a fragmentary diagrammatic view of apparatus, in which the spring filament of the invention may be manufactured.

The elastic filament or filamentous spring of this invention is formed of a strand or wire of metal. The metal is a metal that, initially in relatively ductile condition, may be hardened and rendered resilient, either by "cold working" or by heat treatment, or by both cold working and heat treatment. The metallurgical art is familiar with many metals of this character, and it is needless herein to consider their analyses. Suffice it to say, the metal may be a brass or a bronze, or a Monel metal (a metal consisting principally of brass and nickel); alternately it may be a steel, particularly and preferably a stainless steel, or similar rustless ferrous-base metal. The selection of the particular metal to be used in the manufacture of filaments for a particular device or field of service will depend upon the conditions of service which the elastic filament must withstand, and with such matters as these the invention is not immediately concerned.

The most important aspect of the invention concerns the structural shape of the filament. It is essential that the filament will be highly flexible and resilient, and that it shall retain these characteristics over adequate periods of service. With these requisites in mind, it will be understood that the filament of the invention is, advantageously, a flat filament of serpentine or corrugated structural form. The corrugations may consist either in a single or in a multiple system of corrugations.

Referring to the drawing, the structure of the filamentous spring will be described.

A wire 1, drawn from a supply spool 2, is first corrugated and then it is flattened in the plane 5 of the corrugations. In the course of such "cold working" operations the initially ductile metal body of the wire is work hardened, and a substantial degree of resilience is imparted to such body, providing an elastic filament that embodies the invention. (In the parlance of the art the hardness and resilience may be said to be induced by "cold working" in the attenuated body of metal.) More specifically, the wire (in this case a round steel wire of from .008" to .030" 10 in diameter) is led through a pair of corrugating rolls 3, 4 and is corrugated (as shown at 5), with the corrugations extending in common plane. Upon emerging from such rolls, the corrugated wire 5 is fed flat-wise between a pair of pressure 15 rolls 6, 7, and the rolls 6, 7 operate to compress and spread the body of the wire into a thin elastic ribbon 8. It will be noted that the ribbon-like body of the filament extends flat in the plane of the corrugations, with the effect that the 20 flexibility of the filament is greatest in directions transverse to the plane of the corrugations, and the resilience or spring effect greatest in directions extending in such plane. It will be also noted that the opposite thin edges of the ribbon 25 are presented in the crests of the corrugations, whereby the efficiency of the filament, when made into cutting, scouring, or abrading devices, 30 is of highest order.

The pressure of the rolls 6, 7 may be regulated, 35 such that the thickness and breadth of the body of the filament may be brought to specified values. In practice I have provided the ribbon-like filaments in thicknesses of from .001" to .010", and in breadths of from .015" to .070", 40 but these values are merely given in exemplary way.

The corrugated elastic filament 8 will, without refinement, prove valuable in many fields of use. However, in some cases the resilience and hardness 45 of its metal body may with advantage be modified, say by heat treatment, and thus brought into condition best to meet particular needs. In refinement, the corrugated filament may be further particularly constructed, to increase the 50 characteristics desired. For example, the corrugated filament 8 may be axially twisted, in such manner that the system of corrugations do not extend in common plane, but extend in helical succession with respect to the axis of the filament. Alternately, the filament may be formed

with a second system of corrugations, and it is to be noted that such a doubly corrugated filament provides the preferred or most effective embodiment of the invention.

In the production of such doubly corrugated filament, the singly corrugated filament 8 is passed through a second pair of corrugating rolls 9, 10 and corrugated in transverse direction with respect to the plane of the first corrugations, providing the doubly corrugated filament 11. The entire filament-forming operation may be conducted with continuity of operation; that is, the filament 8 may pass in uninterrupted course from the pressure rolls 6, 7 to the second set of corrugating rolls 9, 10, and, in the course of travel, the filament 8 may be twisted through an angle of 90°, as the dotted arrows indicate in the drawing, and thus brought into proper position for the second pass of corrugating rolls. As is manifest from what has been said, the second or transverse corrugations extend (in this case) at an angle of 90° to the common plane of the corrugations first formed. Of course, in producing this doubly corrugated filament, the metal wire used will be such in character that the elasticity and hardness of the filament 8 will not be so great as to prevent the second or final corrugating and metal-working operations.

I claim as my invention:

1. An article of the class described consisting in a wire or strand of resilient metal formed with two systems or lines of corrugations, the undula-

tions of one system of corrugations being angularly disposed with respect to the undulations of the other system.

2. An elastic filament of the sort described consisting in a thin ribbon of resilient metal corrugated or undulated in the plane of the body of the ribbon, the crests of the corrugations or undulations lying in the thin edges of the ribbon, and such filament having greatest flexibility in a direction extending transversely of the plane in which the corrugations lie, and having in directions extending in such plane greatest resistance to flexure.

3. An elastic filament of the sort described consisting in a thin ribbon of resilient metal corrugated or undulated in the plane of the body of the ribbon, the crests of the corrugations or undulations being formed by the thin edges of the ribbon, and the crests of successive corrugations or undulations being laterally staggered in the line of corrugations or undulations.

4. An article of the class described comprising a flattened, corrugated filament of stainless steel, with the corrugations lying in the plane of the flattened filament, the body of such corrugated filament characterized by a substantial degree of work-induced hardness and elasticity, and the filament having greatest flexibility in a direction extending transversely of the plane in which said corrugations lie.

FRANK C. JACOBS.